

## UNITED STATES PATENT OFFICE.

ARMAND MÜLLER-JACOBS, OF RICHMOND HILL, NEW YORK, ASSIGNOR  
TO COSMOS CHEMICAL COMPANY, A CORPORATION OF NEW YORK.

## PROCESS OF MORDANTING.

SPECIFICATION forming part of Letters Patent No. 769,954, dated September 13, 1904.

Application filed August 19, 1903. Serial No. 170,034. (No specimens.)

*To all whom it may concern:*

Be it known that I, ARMAND MÜLLER-JACOBS, a citizen of the Swiss Republic, and a resident of Richmond Hill, county of Queens, 5 and State of New York, have invented certain new and useful Improvements in Dyeing and Printing Textile or other Fabrics, of which the following is a specification.

My invention relates to dyeing and printing textile fibers or other fabrics; and it consists in the fixation of colors and dyestuffs upon the same in a novel manner, having the advantages of shortening the process of dyeing and printing and gaining at the same time 15 considerably in gloss, brilliancy, durability, and finish in a most expeditious and economical way.

In making experiments I found that if stear-amid is dissolved in appropriate proportions 20 in either soap or turkey-red-oil solutions and anilin colors of either basic or acid character are added to it a liquid is obtained which when applied to cotton, silk, wool, or other fabrics through a padding-machine or by 25 other appropriate means or by printing upon it in the ordinary way the colors can be fixed upon them uniformly and lastingly by steaming or passing the same through hot calenders, in both cases at a temperature of 105° to 110° 30 centigrade. At this temperature the stear-amid melts and fixes mechanically the colors, thereby making it possible to dye mixed goods—such, for instance, as silk and cotton—in one operation without showing any difference 35 in shade of either of the fibers. At the same time it imparts to the goods a certain gloss and finish which is an especial requisite for many of the articles. In some cases a passage through a weak bath of a mineral or organic acid or through a weak bath of a soluble 40 metal salt—as, for instance, sulfate of alumina—may replace the heating, steaming, or calendering and besides may be considerably useful in fastening the colors. Paper, wood, 45 leather, and all other fibrous materials requiring high gloss or sizing can be treated in the same way.

In carrying out my invention I proceed as follows: I dissolve pure stear-amid in a boiling solution of neutral soap or of turkey-red oil, the former to be preferred. One part of either of these substances in a concentrated form is sufficient in combination with two to four parts of the stear-amid to maintain the latter in solution or in an extremely fine emulsion. When diluted with warm water, so that the quantity of stear-amid amounts to five per cent., it is practically in the right state to receive the coloring-matter in shape of watery or alcoholic solutions.

Magenta, methyl-violet, or brilliant green, for instance, as well as azo colors, acid colors, the eosins, &c., are all colors to be used in appropriate quantities for the production of the shades necessary for the impregnation 65 of the goods. For printing purposes thickening materials—such as starch, dextrine, gum-tragacanth, or the like—have to be added to the combined amid and color solution, and for dyeing leather I may simply apply 70 such solutions or emulsions prepared as mentioned above by using a brush or other suitable means. I may also use stear-amid in alcohol, benzole, tetrachlorid of carbon, acetone, &c., solutions with colors that are soluble in 75 the corresponding solvent, and thereby obtain color solutions which can be applied on cotton, silk, and mixed goods or the like directly, the coloring-matter being fixed after evaporation of the solvent by the aid of stear-amid and subsequent heating or steaming processes.

What I claim as my invention is—

In the art of dyeing and printing textile fabrics the method of fixing colors and dyestuffs which consists in acting on said fabrics with a compound containing stear-amid as a mordant or mordanting material.

Signed at New York this 14th day of August, 1903.

ARMAND MÜLLER-JACOBS.

Witnesses:

C. SEDGWICK,  
A. P. THAYER.